

## UNITED STATES PATENT OFFICE

HENRY A. DE FRIES, OF ALBANY, NEW YORK, ASSIGNOR TO LUDLUM STEEL COMPANY, OF WATERVLIET, NEW YORK, A CORPORATION OF NEW JERSEY

## MANUFACTURE OF IRONS AND STEELS

No Drawing.

Application filed April 27, 1928. Serial No. 273,433.

My invention relates to the manufacture of iron and steel and particularly to the development of improved methods of deoxidization whereby the quality of steels and irons is greatly enhanced, and to an improved procedure in the remelting of alloys containing easily oxidizable constituents such as chromium and silicon, for example, whereby scrap steels and irons of such composition may now be advantageously utilized in the manufacture of ferrous alloys.

Various substances either singly or in combination have been used as deoxidizers in the process of making ferrous-alloys. Among those often used is aluminum which is generally added to the molten metal in the ladle or in the ingot mold, and in very rare instances, in the furnace. Aluminum is light, melts at a comparatively low temperature and is readily oxidized. Therefore, when added in the usual way to a molten metal of higher specific gravity and having a much higher melting point, it melts quickly on the surface of the molten metal and, because of its great affinity for oxygen, very quickly picks up oxygen from the air instead of from the molten metal to which it has been added. Because it is readily oxidizable its action in molten steel or iron proceeds very quickly, and if complete deoxidization does not take place almost instantaneously there is great danger that it does not take place at all. Again, where the aluminum is added in the ladle, for example, oxide inclusions are very likely to be present in the final product, due first, to the fact that sufficient time does not elapse for these alumina inclusions to rise to the surface of the molten metal, and second, to the fact that any free aluminum in the steel will be oxidized during the pouring as the molten stream of metal passes through the air. The oxide thus formed is churned into the ingot and appears as crystalline alumina in the finished product. Then too, the aluminum forms a dross which is an ir-

reducible compound of aluminum and alumina. Sometimes this dross gets into the steel and forms inclusions of the worst possible character. The use of aluminum as a deoxidizer is, therefore, always attended with great uncertainty of operation, and the result sometimes is the opposite of that which it was desired to attain.

I find that by using the intermetallic compound  $FeAl_3$ , or an alloy very closely approaching this compound, instead of aluminum alone, the difficulties heretofore attendant upon the use of aluminum in the general manufacture of steel are eliminated. This compound is a great deal heavier than aluminum and its melting point is almost twice as high as aluminum alone. It is brittle and porous so that it can be conveniently added to the molten metal in masses of any size desired. It is a slower deoxidizer than aluminum and is extremely thorough in its action. Because of these characteristics, it may, if desired, be added directly to the molten metal in the furnace, thereby insuring complete deoxidization and complete removal of the alumina and other inclusions into the slag before the melt is poured. As a deoxidizer its action takes place throughout the entire bath instead of at the surface thereof as in the case of aluminum. Generally speaking, it is immaterial at what stage of the manufacturing process the  $FeAl_3$  is added because its beneficial action is continued throughout the melting, pouring and casting, and where a slight excess over and above that necessary to deoxidize the steel is provided, it prevents the metal from going wild in the mold. In addition to functioning as a highly efficient deoxidizer it will be found extremely useful in the general manufacture of ferrous-alloys as hereinafter outlined.

In the manufacture of carbon steel in which carbon is the principal element (aside from iron), it acts as a true deoxidizer when added to the bath in the furnace before pouring.

In the general manufacture of alloy steels the ferro-aluminum may be added to the bath as a deoxidizer before making the alloy addition. In this case the residual aluminum in liquid solution from the ferro-aluminum prevents the alloy addition from oxidizing while being melted in.

In the remelting of easily oxidized metals and scrap, such as chromium, high chromium or silicon steel and iron, any alumina which may form from the oxidation of the aluminum will have time to rise to the surface of the bath and combine with the slag, thus leaving the final product practically free from oxide inclusions.

In the manufacture of chromium-silicon irons or steels, high nickel chromium steels and irons, high nickel, high chromium-silicon steels and irons, or in fact all those various ferrous-alloys which are today classified as heat resisting, stainless steels or irons, the necessary amount of  $FeAl_3$  added to the cold remelting charge or scrap charge will prevent oxidation and will, therefore, keep the carbon content reasonably close to the carbon content of the initial charge. If a building up of alloys is necessary, some additional ferro-aluminum may be added to the bath before the alloys.

In the manufacture of gray iron,  $FeAl_3$  added in the ladle not only fully deoxidizes the iron, thereby making a denser structure, but also effects therein a finer dissemination and a more uniform distribution of graphitic carbon than has heretofore been attainable.

In using ferro-aluminum it is always preferable to add it in as large masses as possible, preferably preheated to about 1000-1500 degrees F. I find that such large masses will melt more uniformly into the bath and be more thoroughly distributed therein. After the ferro-aluminum is melted in, the bath should be stirred vigorously to obtain a thorough mixing.

While many modifications of the procedure herein outlined may be made, I find that the following will give very satisfactory results.

In the manufacture of carbon steel having the following composition, for example—

|               | Per cent  |
|---------------|-----------|
| Carbon        | 1.05-1.15 |
| Manganese     | 0.20-0.30 |
| Silicon       | 0.20-0.30 |
| Phosphorus    | 0.015     |
| Sulphur       | 0.015     |
| Balance iron, |           |

the scrap charge is melted and a sample taken. The steel is then deoxidized by standard deoxidizing slag and the carbon is brought to specification. Ferro-aluminum, preferably preheated, is then melted in and the bath thoroughly stirred. The heat is then held for 10 to 15 minutes to insure deoxidization before pouring. The resulting steel will be free from aluminum oxide because any re-

sidual aluminum therein will be in liquid solution in the molten steel, in which condition it will not oxidize on contact with the air during pouring.

In the manufacture of chromium steel conforming to the following specification, for example—

|               | Per cent  |
|---------------|-----------|
| Carbon        | 0.95-1.05 |
| Manganese     | 0.25-0.35 |
| Silicon       | 0.20-0.30 |
| Chromium      | 1.40-1.50 |
| Balance iron, |           |

the scrap charge is melted down and the regular deoxidizing slag is put on. Sufficient ferro-aluminum is then added not only to deoxidize the steel but to provide a slight excess so that there will be some aluminum in liquid solution in the bath. The chromium is then added and melted in. Where the proper amount of ferro-aluminum is used there will be no change in color or composition of the slag, establishing the fact that no oxidation of the chromium has taken place.

In the making of chromium rustless iron, after making a low carbon melt down to say 0.04%, it has heretofore been found extremely difficult to prevent a considerable carbon increase when melting in the chromium. This is due to the facility with which chromium takes up carbon from the furnace electrodes. Where it is desired, to make a 10,000 pound heat of rustless iron conforming to the following specification, for example—

|                  | Per cent    |
|------------------|-------------|
| Carbon (maximum) | 0.09        |
| Manganese        | 0.50        |
| Silicon          | 0.75-1.00   |
| Chromium         | 16.50-18.50 |

the procedure may be as follows:

Common scrap plus 250 pounds of silico manganese (70% manganese, 20% silicon, 1% carbon) is melted down. 400 pounds of iron ore is added to bring the carbon down to 0.04% and the slag is then pulled. A new slag of lime mixed with fine silicon or ferro-silicon is added for primary deoxidization, then 85 pounds of ferro-aluminum, preferably preheated, is melted in and thoroughly stirred into the bath. The required amount of low carbon ferro-chromium, properly preheated, is then added and melted in, whereupon an additional 15 pounds of ferro-aluminum is added. The final product will be found to contain about 0.08%-0.10% aluminum, but will be practically free from alumina and other oxide inclusions and will show no alligator skin. Furthermore, there will be no appreciable increase in the carbon content which is probably due to the fact that the deoxidizing action of the aluminum in the bath prevents, to a great extent, the absorption of carbon by the chromium while being melted in.

In making a heat of silicon chromium steel conforming to the following specification, for example—

|               | Per cent  |
|---------------|-----------|
| Carbon        | 0.40-0.50 |
| 5 Manganese   | 0.20-0.60 |
| Silicon       | 3.00-3.50 |
| Chromium      | 8.00-9.00 |
| Balance iron, |           |

10 it has been found very difficult to remelt scrap steel of this analysis without excessive losses in chromium and silicon due to oxidation during the melting down. Furthermore, the chromium and silicon oxide produced becomes so thoroughly entrapped in the steel that it has heretofore been practically impossible to remove them with known deoxidizers. I find that the addition of  $FeAl_3$  to the initial charge overcomes this difficulty, and 20 sound steel may be produced using silicon chromium steel scrap only.

For a 10,000 pound heat the procedure is as follows: 75 pounds of  $FeAl_3$  is added to the silicon chromium steel scrap charge and 25 the whole melted down. The melting down slag is removed and new slag added. An additional 25 pounds of  $FeAl_3$  is then added, the necessary alloy additions made, and the heat poured. The losses of chromium and silicon 30 in such a heat is less than 50 points or 0.50% maximum less than the analysis of the original charge.

In the remelting of rustless iron scrap containing 10% to 20% chromium the scrap is charged into the furnace with  $FeAl_3$ . The 35 charge is melted down and the slag removed. A new lime slag mixed with fine ferro-silicon is then put on and a small amount of  $FeAl_3$  is melted in. Following this, the necessary 40 alloy additions are made to make up for the amount lost during the melting down, and the heat is poured.

I am aware that others have heretofore suggested the method of alloying aluminum with steel or iron by pre-alloying the aluminum with iron to form a so-called ferro-aluminum and then incorporating this in the melt. For example, Hadfield, in U. S. Patent No. 461,333, suggests the use of a ferro-aluminum containing 10% of aluminum; Cooper in U. S. Patent No. 1,550,509 suggests the use of a ferro-aluminum containing equal percentages of iron and aluminum to produce an alloy containing between 10% and 16% of aluminum. It has also been suggested by Wittenstrom that castings of wrought iron and steel are improved by the addition of from 0.1% to 0.2% of metallic aluminum.

While my present invention concerns the 60 production of ferrous alloys of superior quality by the use of a ferro-aluminum, it must be borne in mind that the advantageous results herein pointed out cannot be expected unless the ferro-aluminum employed is approximately a true intermetallic compound.

conforming to the formula  $FeAl_3$ , or about 40% iron and 60% aluminum.

In claiming my invention I have used the general term "ferrous alloys" as defining those compositions of matter which are principally iron or which contain a substantial amount of iron combined with one or more other elements.

What I claim is—

1. In the manufacture of iron and steel, 75 the method of deoxidizing the bath which comprises incorporating therewith an alloy of iron and aluminum conforming approximately in composition to the intermetallic compound  $FeAl_3$  and thereafter holding the 80 heat for an appreciable interval before pouring to insure deoxidization.

2. The method of manufacturing a ferrous alloy containing an easily oxidizable element which comprises incorporating in the 85 bath a sufficient quantity of an alloy of iron and aluminum conforming approximately in composition to the intermetallic compound  $FeAl_3$  to effect deoxidization, and thereafter adding the oxidizable element.

3. The method of manufacturing a ferrous alloy containing an easily oxidizable element which comprises creating a liquid solution of aluminum in the bath by incorporating therein an alloy of iron and aluminum conforming 95 approximately in composition to the intermetallic compound  $FeAl_3$ , and in a quantity slightly in excess of that required to effect deoxidization, and thereafter adding the oxidizable element.

4. In the manufacture of ferrous alloys from scrap containing chromium, the method of preventing excessive oxidation of the chromium and the entrapping of chromium oxides in the steel which comprises melting with the scrap charge up to about 1% of an alloy of iron and aluminum approximating in composition the intermetallic compound  $FeAl_3$ .

5. In the manufacture of iron or steel, the 110 method of forming a liquid solution of aluminum in the bath which comprises incorporating therein an alloy of iron and aluminum approximating in composition the intermetallic compound  $FeAl_3$ , and in a quantity slightly 115 in excess of that required for deoxidization.

6. These steps in the manufacture of ferrous alloys containing easily oxidizable elements which comprise effecting a primary deoxidization of the bath, and thereafter completely deoxidizing by the addition of an alloy of iron and aluminum approximating in composition the intermetallic compound  $FeAl_3$  and before making the necessary alloy additions.

7. Those steps in the manufacture of ferrous alloys containing easily oxidizable elements which comprise effecting a primary deoxidization of the bath, completing the deoxidization by the addition of an alloy of

iron and aluminum approximating in composition the intermetallic compound  $FeAl_3$ , making the necessary alloy additions, and thereafter adding an additional quantity of  $FeAl_3$ ; the total quantity of  $FeAl_3$  added being slightly in excess of that required to effect deoxidization.

**HENRY A. DE FRIES.**

**10****15****20****25****30****35****40****45****50****55****60**